



US005120627A

# United States Patent [19]

Nozomi et al.

[11] Patent Number: 5,120,627

[45] Date of Patent: Jun. 9, 1992

[54] ELECTROPHOTOGRAPHIC  
PHOTORECEPTOR HAVING A DIP  
COATED CHARGE TRANSPORT LAYER

[75] Inventors: Mamoru Nozomi, Yokohama;  
Shigenori Otsuka, Omiya; Hiromi  
Horiuchi, Tokyo; all of Japan

[73] Assignee: Mitsubishi Kasei Corporation,  
Tokyo, Japan

[21] Appl. No.: 559,277

[22] Filed: Jul. 30, 1990

[30] Foreign Application Priority Data

Aug. 1, 1989 [JP] Japan ..... 1-99563

[51] Int. Cl.<sup>5</sup> ..... G03G 5/14

[52] U.S. Cl. ..... 430/59; 430/132

[58] Field of Search ..... 430/129, 58, 59, 132

[56] References Cited

U.S. PATENT DOCUMENTS

4,407,919 10/1983 Murayama et al. ..... 430/58

4,943,502 7/1990 Terrell et al. ..... 430/5  
4,943,508 7/1990 Yu ..... 430/12

Primary Examiner—John Goodrow

Attorney, Agent, or Firm—David G. Conlin; Linda M.  
Buckley

[57] ABSTRACT

Disclosed herein is an electrophotographic photoreceptor having on a conductive base at least one charge generation layer and at least one charge transport layer, said charge transport layer having the thickness of 2  $\mu$ m or above and being formed with a coating solution containing a condensation polymer of the viscosity average molecular weight of 15,000 to 25,000 as binder resin according to the dip coating method. The electrophotographic photoreceptor according to the present invention has the excellent durability because the resultant charge transport layer has the increased and uniform thickness without changing the electrical properties, especially the charged potential.

12 Claims, 1 Drawing Sheet

*Fig. 1*

**ELECTROPHOTOGRAPHIC PHOTORECEPTOR  
HAVING A DIP COATED CHARGE TRANSPORT  
LAYER**

**FIELD OF THE INVENTION**

The present invention relates to an electrophotographic photoreceptor. More particularly, it relates to the electrophotographic photoreceptor having an excellent durability.

**BACKGROUND OF THE INVENTION**

In recent years, the electrophotography has been applied to copying machines as well as various printers since they can give images with high qualities without delay. As a photoreceptor which plays an important role in the electrophotography, the photoreceptor comprising an inorganic photoconductive material such as selenium, arsenic-selenium alloy, cadmium sulfide, zinc oxide and the like has been used. More recently, the photoreceptor comprising an organic photoconductive material was proposed. The latter has the advantages which is not a pollutant and which has a film-formability and a shapability.

As one of the organic photoreceptors, the so-called "laminated-type photoreceptor" in which a charge generation layer, the thickness of which is usually about 0.5  $\mu\text{m}$ , and a charge transport layer, the thickness of which is usually about 10 to 20  $\mu\text{m}$ , are successively laminated was developed. The laminated-type photoreceptor is increasingly interested in and is expected to be widely used in the near future because it has the following advantages:

(1) the photoreceptor having high sensitivity can be obtained by suitably selecting and combining the charge generation material and the charge transport material;

(2) the photoreceptor having high safety can be obtained because the charge generation material and the charge transport material can be selected from a wide range of the materials; and

(3) the photoreceptor can be prepared by simple coating and thus it can be prepared with low costs.

In general, a photosensitive layer comprising the charge generation layer and the charge transport layer is formed on a conductive base according to any one of the known methods such as a dip coating method, a spray method, a wire bar method, a blade method, a roller method, a curtain coater method and so on. When the conductive base is an endless pipe, the dip coating method wherein an object to be coated is dipped in a vessel containing a coating solution followed by lifting the object from the surface of the coating solution at a constant speed is usually and preferably employed because it can give a coated film with an uniform thickness relatively easily.

The prior laminated-type photoreceptors are very poor in durability when compared with the inorganic photoreceptors so as to limit their application.

One important cause of such a poor durability is that the thickness of the charge transport layer reduces by being subjected to the abrasion during the cleaning step of the electrophotographic process. The reduction in thickness of the charge transport layer is accompanied by the lowering of the charged potential and thus the lowering of the contrast on the resultant images. As one of the effective means for preventing the reduction in thickness of the charge transport layer, it is proposed to

increase the thickness of the charge transport layer so to prevent the change of the charged potential.

The approach of increasing the thickness of the charge transport layer has two problems. Firstly, the charge transport layer with the increased and uniform thickness cannot be obtained according to the conventional dip coating method because a large volume of the coating solution drop down and the coating cannot be conducted at the suitable speed. For effectively forming the charge transport layer with the increased and uniform thickness according to the dip coating method, the use of the low molecular weight polymer as a binder resin so as to prepare the coating solution having the high solid concentration and the reduced viscosity is considered. However, the abrasion resistance of the charge transport layer is impaired when this coating solution is used, and as the result, the advantage effect by increasing the thickness of the charge transport layer will be compensated.

Secondly, when the thickness of the charge transport layer increases, the photoreceptor has the low optical responsiveness. Because, the increase of the thickness of the charge transport layer weakens the electric field strength which affects the mobility of carriers and the optical responsiveness of the photoreceptor.

An object of the present invention is to provide the electrophotographic photoreceptor having the excellent durability and the excellent electric properties for a long period, which can be easily and efficiently prepared.

The present inventors found that the above object of the present invention can be achieved by forming the thicker charge transport layer with the coating solution containing a specific polymer as the binder resin according to the dip coating method.

**SUMMARY OF THE INVENTION**

The present invention provides the electrophotographic photoreceptor which has on a conductive base at least one charge generation layer and at least one charge transport layer, the charge transport layer having the thickness of 27  $\mu\text{m}$  or above and being formed with the coating solution containing a condensation polymer of the viscosity-average molecular weight of 15,000 to 25,000 as the binder resin according to the dip coating method.

**DETAILED EXPLANATION OF THE INVENTION**

The photoreceptor according to the present invention has the conductive base, on which the photosensitive layer comprising the charge generation layer and the charge transport layer is provided. As the conductive base, any of the known conductive bases usually used in the electrophotographic photoreceptor can be used. Examples of the conductive base include a base made of a metallic material such as aluminium, stainless steel, copper and nickel and a base made of an insulating material such as polyester film or paper which has a conductive layer such as a layer of aluminium, copper, palladium, tin oxide and indium oxide. Among them, an endless pipe of metal such as aluminium is preferable.

A known barrier layer may be provided between the conductive base and the charge generation layer, generally used in the photoreceptor. As the barrier layer, a layer of an inorganic material such as aluminium anodic oxide film, aluminium oxide and aluminium hydroxide or a layer of an organic material such as poly-

yl alcohol, casein, polyvinyl pyrrolidone, polyacrylic acid, celluloses, gelatin, starch, polyurethane, polyimide and polyamide is used.

The charge generation layer comprises a charge generation material and a binder resin. As the charge generation material used in the charge generation layer, various inorganic photoconductive materials such as selenium and its alloys, arsenic-selenium alloy, cadmium sulfide and zinc oxide or various organic pigment or dye such as phthalocyanine, azo, quinacridone, polycyclic quinone, pyrylium salt, thiapyrylium salt, indigo, thionigo, anthoanthrone, pyranthrone and cyanine can be used. Among them, phthalocyanine without metal, phthalocyanines coordinated with metal or its compound such as copper, indium chloride, gallium chloride, tin, oxytinanium, zinc and vanadium, azo pigments such as monoazo, bisazo, trisazo and polyazo are preferable.

As the binder used together with the charge generation material in the charge generation layer, any of the binder resins usually used in the charge generation layer can be used. Examples of the resins include resins such as polyvinyl acetate, polyacrylate, polymethacrylate, polyester, polycarbonate, polyvinyl acetal, polyvinyl propional, polyvinyl butyral, phenoxy resin, epoxy resin, urethane resin, cellulose ester and cellulose ether.

The charge generation material is used in an amount of 20 to 300 parts by weight, preferably 30 to 200 parts by weight per 100 parts by weight of the binder resin.

If necessary, the charge generation layer may contain various additives such as a leveling agent, an antioxidant and a sensitizer.

The thickness of the charge generation layer is generally 0.1 to 1  $\mu\text{m}$ , preferably 0.15 to 0.6  $\mu\text{m}$ .

The charge generation layer can be formed on the conductive base according to any one of the known methods, preferably the dip coating method.

The charge transport layer comprises a charge transport material and a binder resin.

As the charge transport material used together with the binder resin in the charge transport layer, high mo-

lecular weight compounds such as polyvinyl carbazole, polyvinyl pyrene and polyacenaphthylene and low molecular weight compounds such as pyrazoline derivatives, oxazole derivatives, hydrazone derivatives, stilbene derivatives and amine derivatives are exemplified.

In the charge transport layer according to the present invention, the condensation polymer is used as the binder resin. The condensation polymer used should have the viscosity-average molecular weight of 15,000 to 25,000. Herein the viscosity-average molecular weight of the polymer is calculated from the following equation.

$$[\eta] = K[Mv]^{\alpha}$$

wherein

$Mv$  is viscosity-average molecular weight,

$\eta$  is intrinsic viscosity,

$K$  and  $\alpha$  are constants depending on the natures of polymer and solvent used and the determination temperature. When the condensation polymer having the viscosity-average molecular weight ( $Mv$ ) of less than 15,000 is used, the mechanical strength of the polymer itself is very low and thus the resultant charge transport layer has the poor abrasion resistance. On the other hand, when the condensation polymer having the viscosity-average molecular weight ( $Mv$ ) of above 25,000 is used, the problems such as that the coating speed for obtaining the coated film with the desired thickness is very slow, that the times required for coating is very long and that the thickness of the coated film is not uniform are caused.

As the condensation polymer usable in the present invention, resins of polycarbonate, polyester, polysulfone, polyether, polyketone, polyimide, polyester carbonate, polybenzimidazole, polyether ketone, phenoxy and epoxy are exemplified. Among them, polycarbonate, polyester and/or polyester carbonate resins having repeating units which are represented by the following formulas (I) to (IV) are preferable with respect to electric properties.



-continued



In the above formulas, R<sup>1</sup> and R<sup>2</sup> are independently hydrogen atom, alkyl group containing 1 to 3 carbon atoms, trifluoromethyl group or phenyl group. Alternatively, R<sup>1</sup> together with R<sup>2</sup> may form cycloalkylidene group such as cyclohexylene. R<sup>3</sup>, R<sup>4</sup>, R<sup>5</sup> and R<sup>6</sup> are independently hydrogen atom, halogen atoms or alkyl group containing 1 to 3 carbon atoms. R<sup>7</sup> is a residue of divalent acid such as terephthalic acid, isophthalic acid, 2,6-naphthalenedicarboxylic acid and diphenic acid. R<sup>8</sup>

15

is alkylene group containing 2 to 6 carbon atoms or 2,2-bis(4-hydroxycyclohexyl)propane.

10 The preferably repeating units in the condensatic polymer are shown below. In the formulas,



represents para- or meta-substitution.

polycarbonate resin

(IV)

-continued

polyester resin

-continued





-continued



These condensation polymers may be homopolymers or copolymers copolymerized with other comonomers. Alternatively, the condensation polymer may be used in a mixture with other condensation polymer(s). In the polyester carbonate resins, the ratios of carbonate components to ester components can be freely and suitably varied.

The charge transport material is generally used in an amount of 30 to 200 parts by weight, preferably 50 to 150 parts by weight per 100 parts by weight of the binder resin.

If necessary, the charge transport layer may contain various additives such as an antioxidant, a sensitizer and a levelling agent.

The thickness of the charge transport layer should be at least 27  $\mu\text{m}$ . Preferably, it is 30 to 50  $\mu\text{m}$ .

The charge transport layer is prepared on the charge generation layer according to the dip coating method. For this purpose, the coating solution containing the charge transport material, the binder resin and optionally the additives in a solvent is used. It is preferable for efficiently obtaining the charge transport layer with the uniform thickness to use the coating solution preferably having the solid concentration of 25% or above and preferably not more than 35% and having the viscosity of 50 to 300 cPs, preferably 50 to 200 cPs. As the solvent used, the solvent having the boiling point of 35 to 150°C. is preferable since it can be air-dried at a suitable speed. Examples of the suitable solvents are mentioned below. Aromatic hydrocarbons such as benzene, tolu-

ene and xylene; ketones such as acetone, methyl ethyl ketone, diethyl ketone, methyl isobutyl ketone, cyclohexanone and cyclopentanone; esters such as methyl acetate, methyl propionate, methyl cellosolve and ethyl cellosolve; alcohols such as methanol, ethanol, propyl alcohol and butanol; ethers such as tetrahydrofuran, dioxane, dimethoxymethane, dimethoxyethane and diglym; halogenated hydrocarbons such as carbon tetrachloride, chloroform, methylene chloride, dichloroethane, trichloroethane and chlorobenzene; amides such as N,N-dimethylformamide and N,N-dimethylacetamide; and dimethylsulfoxide. The solvent may be used in a mixture.

In the preparation of the charge transport layer according to the dip coating method, the coating speed is controlled so as to obtain the coated film with the thickness of 27  $\mu\text{m}$  or above, preferably 30 to 50  $\mu\text{m}$ . Here the coating speed means the speed of lifting the object to be coated from the surface of the coating solution. About 30 to 80 cm/min is suitable. When the coating speed is less than about 30 cm/min, the satisfactory productivity cannot be achieved. On the other hand, when the coating speed is above 80 cm/min, the coated film with the uniform thickness cannot be obtained due to the effect of the vibration of the coating apparatus.

## EXAMPLES

The invention will be better understood by reference to certain examples, which are included herein for purposes of illustration.

oses of illustration only and are not intended to limit  
the invention.

## EXAMPLE 1

10 parts by weight of a bisazo compound having the following formula:



as added to 150 parts by weight of 4-methoxy-4-ethylpentanone-2 and they were subjected to the binding and dispersion treatment with a sand grind mill. The thus obtained dispersion was added to 200 parts by weight of a 5% solution of 1,2-dimethoxyethane in polyvinyl butyral (#6000-C (trade name), ex ENKI KAGAKU KOGYO KABUSHIKI KAI-HA) so as to prepare a dispersion with the solid concentration of 4.0%.

In the above dispersion, an aluminium cylinder having a mirror finished surface and having the outer diameter of 80 mm, the length of 340 mm and the thickness of 1.0 mm was dipped and a charge generation layer was coated on the aluminium cylinder to provide a dried film with the thickness of 0.3  $\mu$ m.

Then, this aluminium cylinder was dipped in a coating solution at the coating speed of 40 cm/min so as to coat the charge transport layer on the charge generation layer. The coating solution contained 95 parts by weight of a hydrazone compound having the following formula:



5 parts by weight of a cyano compound having the following formula:



and 100 parts by weight of polycarbonate resin having a viscosity-average molecular weight of 24,400 and the following repeating unit:



in a mixed solvent of dioxane and tetrahydrofuran and had the solid concentration of 27.5% and the viscosity of 195 cPs. The charge transport layer was dried at room temperature for 30 minutes and 125° C. for 20 minutes to provide a dried film with the thickness of 32  $\mu$ m.

The distribution in thickness of the charge transport layer from the edge where was firstly lifted from the coating solution was determined. The result is shown in FIG. 1. Its ordinate is a distance from the edge and its abscissa is the thickness of the coated film. As shown in FIG. 1, the charge transport layer at 20 mm from the edge had the thickness corresponding to 95% of the average. From this result, it can be said that the charge transport layer having the uniform thickness could be obtained efficiently according to the present invention.

## EXAMPLE 2

The procedure of Example 1 was repeated, except that the coating solution for the charge transport layer which contained the polycarbonate resin of the viscosity-average molecular weight of 20,300 and had the solid concentration of 30% and the viscosity of 120 cPs was used so as to provide the dried film of the charge transport layer with the thickness of 40  $\mu$ m. Then, the coating speed was controlled to be 48 cm/min.

The charge transport layer at 18 mm from the edge had the thickness corresponding to 95% of the average.

## COMPARATIVE EXAMPLE 1

The procedure of Example 1 was repeated, except that the coating solution for the charge transport layer which contained the polycarbonate resin of the viscosity-average molecular weight of 31,000 and had the solid concentration of 30% and the viscosity of 520 cPs was used so as to provide the dried film of the charge transport layer with the thickness of 40  $\mu$ m. Then, the coating speed was controlled to be 18 cm/min and the long coating period was required.

The charge transport layer at 25 mm from the edge had the thickness corresponding to 95% of the average.

## COMPARATIVE EXAMPLE 2

The procedure of Example 1 was repeated, except that the coating solution for the charge transport layer which contained the polycarbonate resin of the viscosity-average molecular weight of 31,000 and had the solid concentration of 23% and the viscosity of 120 cPs was used so as to provide the dried film of the charge transport layer with the thickness of 40  $\mu\text{m}$ . Then, the coating speed was controlled to be 200 cm/min.

The charge transport layer at 120 mm from the edge had the thickness corresponding to 95% of the average.

It was observed that a large volume of the coating solution dropped down.

## COMPARATIVE EXAMPLE 3

The procedure of Example 1 was repeated, except that the coating solution for the charge transport layer which contained the polycarbonate resin of the viscosity-average molecular weight of 31,000 and had the solid concentration of 23% and the viscosity of 120 cPs was used so as to provide the dried film of the charge transport layer with the thickness of 20  $\mu\text{m}$ . Then, the coating speed was controlled to be 56 cm/min.

The charge transport layer at 18 mm from the edge had the thickness corresponding to 95% of the average.

## EXAMPLE 3

The procedure of Example 1 was repeated, except that the coating solution for the charge transport layer which contained the polyester resin having the viscosity-average molecular weight of 22,000 and the following repeating unit:



and had the solid concentration of 27% and the viscosity of 110 cPs was used so as to provide the dried film of the charge transport layer with the thickness of 35  $\mu\text{m}$ . Then, the coating speed was controlled to be 40 cm/min.

The charge transport layer at 22 mm from the edge had the thickness corresponding to 95% of the average.

## EXAMPLE 4

The procedure of Example 1 was repeated, except that the coating solution for the charge transport layer which contained the polyester carbonate resin having the viscosity-average molecular weight of 24,100 and the following repeating unit:



and has the solid concentration of 26% and the viscosity of 120 cPs was used so as to provide the dried film of the

charge transport layer with the thickness of 35  $\mu\text{m}$ . Then the coating speed was controlled to be 3 cm/min.

The charge transport layer at 24 mm from the edge had the thickness corresponding to 95% of the average.

## EXAMPLE 5

The procedure of Example 1 was repeated, except that the coating solution for the charge transport layer which contained the polyester resin having the viscosity-average molecular weight of 18,000 and the following repeating unit:



and had the solid concentration of 32% and the viscosity of 80 cPs was used so as to provide the dried film of the charge transport layer with the thickness of 45  $\mu\text{m}$ . Then the coating speed was controlled to be 5 cm/min.

The charge transport layer at 15 mm from the edge had the thickness corresponding to 95% of the average.

## EXAMPLE 6

10 parts by weight of oxytitanium phthalocyanine was added to 150 parts by weight of 4-methoxy-methylpentanone-2 and they were subjected to the grinding and dispersion treatment with a sand grain mill. The thus obtained dispersion was added to 10 parts by weight of a 5% solution of 1,2-dimethoxyethane in polyvinyl butyral (#6000-C (trade name), e.g. DENKI KAGAKU KOGYO KABUSHIKI KAISHA) while applying the ultrasonic (29 KHz) so as to prepare a dispersion with the solid concentration of 4.0%.

In the above dispersion, an aluminium cylinder having a mirror finished surface and having the outer diameter of 30 mm, the length of 260 mm and the thickness of 0.75 mm was dipped and a charge generation layer was coated on the aluminium cylinder to provide dried film with the thickness of 0.3  $\mu\text{m}$ .

Then, this aluminium cylinder was dipped in the coating solution used in Example 2 at the coating speed of 40 cm/min so as to coat the charge transport layer on the charge generation layer. The charge transport layer was dried at room temperature for 30 minutes and 120°C. for 20 minutes to provide a dried film with the thickness of 32  $\mu\text{m}$ .

The charge transport layer at 14 mm from the edge had the thickness corresponding to 95% of the average.

### EXAMPLES 7 TO 9

The procedure of Example 1 was repeated, except that the charge transport material shown in Table 1 was used in place of the hydrazone compound and the cyano compound. 5

TABLE 1

| Ex. | charge transport material                                                          | solid concentration | viscosity |
|-----|------------------------------------------------------------------------------------|---------------------|-----------|
| 7   |   | 27.5%               | 195 cPs   |
|     | 100 parts by weight                                                                |                     |           |
| 8   |   | 27.5%               | 196 cPs   |
|     | 80 parts by weight                                                                 |                     |           |
|     |   |                     |           |
|     | 20 parts by weight                                                                 |                     |           |
| 9   |  | 27.5%               | 196 cPs   |
|     | 100 parts by weight                                                                |                     |           |

The coating speed and the distance from the edge here had the thickness corresponding to 95% of the average in each Examples are shown in Table 2. From this result, it can be said that the charge transport layer having the uniform thickness could be obtained efficiently according to the present invention. It was observed that the dropping of the coating solution was little.

TABLE 2

| Ex. | coating speed | distance from the edge |
|-----|---------------|------------------------|
| 7   | 38 cm/min     | 18 mm                  |
| 8   | 40 cm/min     | 20 mm                  |
| 9   | 40 cm/min     | 20 mm                  |

## TEST EXAMPLE

The photoreceptors prepared in Example 2 and Comparative Example 3 were subjected to the practical copying operation using the commercial copying machine (ex Sharp Corporation, SF-8200). The background potential, the initial potential and the thickness

of the charge transport layer (CTL) were determined. After the copying operation was repeated 20,000 times, the same determinations were carried out. The results are shown in Table 3.

TABLE 3

---

|                                 | Example 2 |                    | Comparative Example 3 |                    |
|---------------------------------|-----------|--------------------|-----------------------|--------------------|
|                                 | initial   | after 20,000 times | initial               | after 20,000 times |
| initial potential (V)           | 700       | 610                | 700                   | 490                |
| background potential (V)        | 20        | 65                 | 15                    | 55                 |
| CTL thickness ( $\mu\text{m}$ ) | 40        | 35                 | 20                    | 15                 |

As clear from the results in Table 3, the reduction in thickness of the charge transport layer was very small according to the present invention and as the result, the photoreceptor according to the present invention has the excellent electric properties during long period.

## EFFECT OF THE INVENTION

The electrophotographic photoreceptor according to the present invention can have the charge transport layer with the increased and uniform thickness owing to the use of the specific binder polymer in the charge transport layer. According to the present invention, the

above charge transport layer can be prepared very efficiently owing to the use of the conventional dip coating method. In addition, the photoreceptor according to the present invention has the excellent durability because the charge transport layer has the sufficient abrasion resistance and therefore, when the photoreceptor is repeatedly used, the reduction in the thickness of the charge transport layer is very little and the change in the electric properties, especially the charged potential is very small.

What is claimed is:

1. A method for preparation of an electrophotographic photoreceptor which has on a conductive base at least one charge generation layer and at least one charge transport layer, characterized in that said charge transport layer is formed into a thickness of 27  $\mu\text{m}$  or above according to a dip coating method with a coating solution which contains a condensation polymer of the viscosity-average molecular weight of 15,000 to 25,000 as a binder resin, the solid concentration of which is 25% or more and the viscosity of which is 50 to 300 cPs.

2. The method according to claim 1, wherein the condensation polymer is at least one resin selected from the group consisting of polycarbonate, polyester, polysulfone, polyether, polyketone, polyimide, polyester carbonate, polybenzimidazole, polyether ketone, penoxy and epoxy.

3. The method according to claim 2, wherein the condensation polymer is polycarbonate, polyester and/or polyester carbonate resin having repeating units which are represented by the following formulas (I) to (IV);



(I)



(II)



(III)



(IV)

wherein  $\text{R}^1$  and  $\text{R}^2$  are independently hydrogen atom, alkyl group containing 1 to 3 carbon atoms, trifluoromethyl group or phenyl group, or alternatively  $\text{R}^1$  together with  $\text{R}^2$  may form cycloalkylidene group;  $\text{R}^3$ ,  $\text{R}^4$ ,  $\text{R}^5$  and  $\text{R}^6$  are independently hydrogen atom, halo-

gen atoms or alkyl group containing 1 to 3 carbon atoms;  $\text{R}^7$  is a residue of divalent acid; and  $\text{R}^8$  is alkylene group containing 2 to 6 carbon atoms or 2,2-bis(4-hydroxycyclohexyl)propane.

4. The method according to claim 1, wherein the charge transport layer has the thickness of 30 to 50  $\mu\text{m}$

5. The method according to claim 1, wherein the solid concentration of the coating solution is 35% or less.

10. The method according to claim 1, wherein the viscosity of the coating solution is 50 to 200 cPs.

7. The method according to claim 1, wherein the coating speed of the coating solution is 30 to 80 cm/mir

15. The method according to claim 1, wherein the charge transport layer contains a charge transport material selected from the group consisting of polyvinyl carbazole, polyvinyl pyrene, polyacenaphthylene pyrazoline derivative, oxazole derivative, hydrazon derivative, stilbene derivative and amine derivative.

9. The method according to claim 1, wherein the charge transport layer comprises a charge transport material and the binder resin and the amount of the charge transport material is 30 to 200 parts by weight per 100 parts by weight of the binder resin.

10. The method according to claim 9, wherein the amount of the charge transport material is 50 to 15 parts by weight per 100 parts by weight of the binder resin.

11. The method according to claim 1, wherein the coating solution contains a solvent having a boiling point of 35° to 150° C.

12. The method according to claim 11, wherein the

65 solvent is aromatic hydrocarbons, ketones, esters, alcohols, ethers, halogenated hydrocarbons, amides or dimethylsulfoxide.

\* \* \* \* \*

UNITED STATES PATENT AND TRADEMARK OFFICE  
CERTIFICATE OF CORRECTION

PATENT NO. : 5,120,627

DATED : June 9, 1992

INVENTOR(S) : Nozomi et al.

It is certified that error appears in the above-identified patent and that said Letters Patent is hereby corrected as shown below:

ON TITLE

PAGE: item [30] replace "1-99563" with --1-199563--

Signed and Sealed this

Seventh Day of September, 1993

Attest:



BRUCE LEHMAN

Attesting Officer

Commissioner of Patents and Trademarks